

# United States Patent

[19]

Nestor

[11] 3,914,934

[45] Oct. 28, 1975

[54] **LOW TEMPERATURE HIGH FLASH POINT  
TURBINE ENGINE FUEL**

3,177,653 4/1965 Barnes et al. .... 60/208

[75] Inventor: **Leonard J. Nestor**, Philadelphia, Pa.

*Primary Examiner*—Samuel Feinberg

[73] Assignee: **The United States of America as  
represented by the Secretary of the  
Navy**, Washington, D.C.

*Attorney, Agent, or Firm*—R. S. Sciascia; Henry  
Hansen

[22] Filed: **Nov. 28, 1973**

[57]

## ABSTRACT

[21] Appl. No.: **419,565**

A turbine engine fuel having a high flash point and low viscosity at -60°F comprising a blend of two to twenty percent by volume of a C<sub>10</sub> or higher alkyl benzene and the remaining volume consisting of a hydrogenated naphtha oil fraction. The fraction is obtained by taking a naphtha fraction from the crude and hydrogenating the naphtha fraction to reduce aromatics. Aromatics containing ten or more carbon atoms are then added to the naphtha fraction.

[52] U.S. Cl. .... 60/208

**8 Claims, No Drawings**

[51] Int. Cl.<sup>2</sup> .... **C06D 5/00**

[58] **Field of Search** .... 60/208, 39.02, 39.06;  
149/108.8, 50; 44/80

[56] **References Cited**

UNITED STATES PATENTS

3,105,351 10/1963 Stahly .... 44/80

## LOW TEMPERATURE HIGH FLASH POINT TURBINE ENGINE FUEL

### STATEMENT OF GOVERNMENT INTEREST

The invention described herein may be manufactured and used by or for the Government of the United States of America for governmental purposes without the payment of any royalties thereon or therefor.

### BACKGROUND OF THE INVENTION

This invention relates generally to the field of fuels and more particularly to a turbine engine fuel having a high flash point and low viscosity.

In developing a fuel for a new Naval missile, called a Harpoon missile, propelled by a gas turbine engine and launched from carrier based Naval aircraft, two fuel property characteristics are essential. Since the missiles are stored aboard Naval vessels, safety regulations require that the fuel have a flash point in excess of 140°F. Engine specifications further require that the fuel have a viscosity less than 12 centistokes at -60°F to allow the engine to start at high altitudes. Exhaustive surveys made of available fuels indicate that the first two requirements could not be met by existing known fuels. Neither JP-4 nor JP-5 type fuels, commonly in

percent by volume of a hydrogenated naphtha oil fraction, and a C<sub>10</sub> or higher alkyl benzene comprising from 2 to 20 percent by volume of the combination of the solvent and the alkyl benzene, the blended fuel having a flash point in excess of 140°F and a maximum viscosity of 12 centistokes at -60°F.

### DESCRIPTION OF THE PREFERRED EMBODIMENT

10 A general physical property rule for fuels is the higher the flash point the higher the viscosity. It is further recognized that a fuel having the desired properties could be produced by blending pure compounds or by using narrow cut fractions of selected jet fuels. However, these approaches are not only complex and difficult to implement, but they also involve extraordinary expense. Since naphthenes tend to have comparatively low viscosities, a survey of products derived from high naphthenic crudes discloses several solvents that have 15 good freeze points, comparatively low viscosities at low temperatures and high flash points. Three such solvents are Kerr Magee Corporation Napoleum 140 solvent, Ashland Chemical Company 140 solvent, and Union Oil Company Amsco 140 solvent, all of whose properties are listed in Table 1.

TABLE 1

| PROPERTY                           | NAPOLEUM<br>140 | ASHLAND<br>140 | AMSCO<br>140 | TEST METHOD*      |
|------------------------------------|-----------------|----------------|--------------|-------------------|
| API Gravity at 60°F                | 45.7            | 46.5           | 49.6         | D-287             |
| Specific Gravity at 60°F           | 0.7985          | 0.7949         | 0.781        | —                 |
| Pounds Per Gallon at 60°F          | 6.648           | 6.62           | 6.51         | —                 |
| Color, Saybolt                     | +30             | +30            | +30          | D-156             |
| Flash Point, °F, TCC               | 145             | 142            | 142          | D-56              |
| Kauri-Butanol Value                | 35              | 37.1           | 30           | D-1133            |
| Araline Point, °F                  | 145             | 138.2          | 164          | D-1012            |
| Distillation, °F                   |                 |                |              | D-86              |
| Initial Boiling Point              | 372             | 368            | 366          | —                 |
| 10%                                | 376             | 372            | 374          | —                 |
| 50%                                | 380             | 375            | 380          | —                 |
| 90%                                | 389             | 380            | 393          | —                 |
| Dry Point                          | 400             | 386            | 405          | —                 |
| End Point                          | 405             | 390            | 406          | —                 |
| Composition - Volume %             | —               | —              | —            | —                 |
| Parafins                           | 48.4            | 55.2           | 53           | Mass Spectroscopy |
| Olefins                            | —               | 0.3            | —            | —                 |
| Naphthenes                         | 47.7            | 35.4           | 47           | Mass Spectroscopy |
| Aromatics                          | 3.9             | 9.1            | <1           | D-1319            |
| Refractive Index at 77°F           | —               | 1.4405         | —            | D-1218            |
| Heat of Combustion-FIA-BTU/LB.     | —               | 18,660         | —            | —                 |
| Sulfur, PEM                        | —               | —              | 1            | D-1266            |
| Acidity of Distillation<br>Residue | —               | Neutral        | —            | D-1093            |
| Corrosion-During Distillation      | 2A              | 1A             | 1A           | D-130             |

\*Indicates ASTM Test Procedure

use for gas turbine engines, meet the necessary requirements. JP-4 fuel, which has a relatively low viscosity at low temperatures, has a flash point below 140°F, and JP-5 fuel, which has a flash point about 140°F and is approved for Naval use, has a viscosity in excess of engine requirements at -60°F.

### SUMMARY OF THE INVENTION

Accordingly, it is a general purpose and object of the present invention to provide a relatively inexpensive fuel suitable for use in a gas turbine engine, and having a flash point in excess of 140°F and a viscosity less than 12 centistokes at -60°F.

These and other objects are accomplished according to the present invention by a blended fuel consisting essentially of a paraffinic solvent containing at least 35

As noted in the table, these solvents contain at least 35% naphthenes and 48% parafins.

55 To support the applicability of high naphthenic crudes to fill the present fuel requirements of the Harpoon missile, a routine sample of JP-5 fuel was obtained from such a crude. Its viscosity was determined to be 18 centistokes at -60°F, somewhat lower than comparable viscosities of JP-5 fuels produced from non-naphthenic crudes. The relatively low viscosity at this temperature was attributed to a high content of naphthenic hydrocarbons.

60 As a class, the aromatics have the lowest viscosities of all hydrocarbons. By blending the aromatic solvents with a low viscosity naphthenic aliphatic solvent, it was theorized that the viscosity requirement could be met while still remaining within a 25% aromatic limitation

also required in the JP-5 fuel specification used by the Navy.

Temperature-viscosity relationships of alkyl benzenes reveal them to be ideally suited as blending agents in order to achieve the desired fuel properties. The relationship between total number of carbon atoms of the alkyl benzenes, and their respective flash points is such that only alkyl benzenes having at least ten total carbon atoms ( $C_{10}$ ) will satisfy the flash point requirement of 140°F or higher. However, pure  $C_{10}$ 's are relatively expensive, ranging in price from \$10 per gallon to \$100 per gallon. The least expensive  $C_{10}$  is secondary butyl benzene costing approximately \$10 per gallon. In order to keep fuel cost down and remain within a 25% aromatic content limitation, blending was deemed desirable.

In testing various combinations of pure materials, several fuels meeting the desired requirements were obtained. The following examples are presented for purposes of illustration and not of limitation.

#### EXAMPLE 1

A composition of fuel comprising 80% by volume of Ashland 140 solvent blended with 20% by volume of secondary butyl benzene (one of a group of  $C_{10}$  alkyl benzenes) was produced using standard blending techniques. The blended fuel had a flash point of 142°F (determined by ASTM D-93 Test Procedure) and a viscosity of 10.6 centistokes at -60°F (determined by ASTM D-445 Test Procedure). Sea level starting tests were conducted at low temperatures using the present blend of fuel on an AiResearch model GTC 85-116 auxilliary power unit (APU), which has a gas turbine engine similar to that used in the Harpoon missile. Sea level starting of the APU was achieved at an ambient temperature of -64°F (viscosity - 11.8 centistokes). In comparison tests with JP-4 fuel it was determined that the time required to attain idle speed of the APU was slightly less with the present blended fuel.

#### EXAMPLE 2

A composition of fuel comprising 98% by volume of Napoleum 140 blended with 2% by volume of secondary butyl benzene was produced as in Example 1. The blended fuel had a flash point of 152°F, and a viscosity of 12.0 centistokes at -60°F determined as in Example 1. Starting tests with the APU yielded results similar to Example 1.

#### EXAMPLE 3

A composition of fuel comprising 87% by volume of Ashland 140 solvent blended with 13% by volume of secondary butyl benzene was produced as in Example 1. The blended fuel had a flash point of 145°F, and a viscosity of 11.8 centistokes at -60°F determined as in Example 1. Starting tests with the APU yielded results similar to Example 1.

#### EXAMPLE 4

A composition of fuel comprising 87% by volume of Amoco 140 solvent blended with 13% by volume of secondary butyl benzene was produced as in Example 1. The blended fuel had a flash point of 152°F, and a viscosity of 12.0 centistokes at -60°F determined as in Example 1. Starting tests with the APU yielded results similar to Example 1.

Studies made with other pure  $C_{10}$  alkyl benzenes, such as iso butyl benzene and normal butyl benzene, indicates that blending them with any of the 140 solvents disclosed herein would yield successful results similar to those reported in Examples 1-4. This conclusion is based upon careful comparison of their properties with those of secondary butyl benzene and published test results of their performance.

Having thus described the present invention, some of the many advantages should now be readily apparent. By blending techniques which are well known to those skilled in the art the applicant has produced a relatively inexpensive family of fuels having viscosities of less than 12 centistokes at -60°F, making them suitable for use in a gas turbine engine operating in extremely low environmental temperatures. The blended fuels further possess the desirable property of having flash points in excess of 140°F, making them safe for storage aboard naval vessels. Heretofore, these properties have been deemed inconsistent with each other and unavailable in a relatively inexpensive fuel.

Obviously, many modifications and variations of the present invention are possible in light of the above teachings. It is therefore to be understood that within the scope of the appended claims the invention may be practiced otherwise than as specifically described.

What is claimed is:

1. A blended fuel suitable for turbine engines consisting essentially of:
  - a paraffinic solvent containing at least 35 percent by volume of a hydrogenated naphtha oil fraction; and an alkyl benzene having at least 10 carbon atoms comprising from 2 to 20 percent by volume of the combination of said solvent and said alkyl benzene, selected from the group consisting of secondary butyl benzene, iso butyl benzene and normal butyl benzene;
  - whereby the blended fuel has a flash point in excess of 140°F and a maximum viscosity of 12 centistokes at -60°F.
2. A fuel as set forth in claim 1 wherein said alkyl benzene is secondary butyl benzene.
3. A fuel as set forth in claim 1 wherein said alkyl benzene is iso butyl benzene.
4. A fuel as set forth in claim 1 wherein said alkyl benzene is normal butyl benzene.
5. The process of operating a gas turbine engine which comprises the steps of:
  - feeding a mixture of air and a fuel consisting essentially of a paraffinic solvent containing at least 35 percent by volume of a hydrogenated naphtha oil fraction, and an alkyl benzene having at least 10 carbon atoms comprising from 2 to 20 percent by volume of the combination of said solvent and said alkyl benzene, selected from the group consisting of secondary butyl benzene, iso butyl benzene and normal butyl benzene, the blended fuel having a flash point in excess of 140°F and a maximum viscosity of 12 centistokes at -60°F, to a chamber;
  - subjecting said mixture to combustion; passing the resulting hot combustion gases through a turbine to partially expand the gases therein; and
  - discharging the hot gases into the atmosphere through a nozzle to produce thrust.
6. A process as set forth in claim 5 wherein said alkyl benzene is secondary butyl benzene.
7. A process as set forth in claim 5 wherein said alkyl benzene is iso butyl benzene.
8. A process as set forth in claim 5 wherein said alkyl benzene is normal butyl benzene.

\* \* \* \* \*